

1

3,265,475

## BUFFING COMPOSITIONS

Donald H. Schantz, Grand Rapids, Mich., assignor, by  
mesne assignments, to Hanson-Van Winkle-Munning  
Company, a corporation of New Jersey  
No Drawing. Filed Dec. 4, 1962, Ser. No. 242,106  
9 Claims. (Cl. 51—304)

This invention relates to buffing compositions and, more particularly, to both non-aqueous and aqueous buffing and polishing compositions which may be easily and completely removed from a metal workpiece by an aqueous alkaline cleaning solution. The invention is based upon the discovery that either aluminum or zinc powder, when incorporated in minor amounts in either a non-aqueous or an aqueous buffing composition, are capable of generating sufficient hydrogen gas when a metal workpiece containing the composition is subsequently cleaned with a hot aqueous alkaline cleaner, thereby aiding in the easy and complete removal of the last traces of the buffing composition remaining after the workpiece has been buffed or polished.

Polishing and buffing compositions generally consist of a carrier lubricant, such as various greases, oils or soaps (compounded to give the desired melting point or viscosity), in which there is dispersed one or more abrasive materials. When a metal workpiece is buffed or polished with these compositions, the residual buffing compound frequently becomes lodged or impacted in the recessed areas, fine lines, scratches or holes in the workpiece, and is quite difficult to remove even when the workpiece is subsequently submerged or scoured with an aqueous alkaline cleaning solution. Oftentimes, the residual buffing composition adheres to the metal surface so tenaciously that even flat surfaces are difficult to clean. Treatment of the polished or buffed metal workpiece with a hot aqueous alkaline cleaning solution is almost always necessary to remove the last traces of the buffing compositions, especially if the polished or buffed workpiece is to be plated. Failure to remove the last traces of such buffing composition from the workpiece invariably leads to imperfect plating.

Using non-aqueous and aqueous buffing compositions both of which comprise a carrier lubricant in which there is dispersed a major amount of an inorganic abrasive, I have found that by incorporating a minor amount of either aluminum powder or zinc powder in this buffing composition, it is possible to prepare an improved buffing composition within which sufficient hydrogen gas may be generated in situ when a metal workpiece containing the composition is subsequently cleaned with hot aqueous alkaline cleaner, thereby aiding in the easy and complete removal of the last traces of buffing composition remaining after the workpiece has been buffed or polished. Based on this discovery, the invention provides an improved buffing composition comprising a carrier lubricant in which there is dispersed a major amount of an inorganic abrasive and a minor amount of metallic powder selected from the group consisting of aluminum and zinc.

In general, only relatively minor amounts of either aluminum or zinc powder (or both) are required in the buffing composition to aid in the removal of the last traces of the composition when the workpiece is subsequently cleaned with an aqueous alkaline cleaning solution. Excellent results have been obtained by using from about  $\frac{1}{2}$  to about 2 percent by weight of the metallic powder (preferably in the form of flakes) in the buffing composition, although for most purposes concentration of the metallic powder in the range from about  $\frac{1}{2}$  to about 1 percent by weight of the composition will suffice.

After the metal workpiece has been buffed and polished with a buffing composition containing either aluminum

2

or zinc powder in accordance with the invention, it may be cleaned with an aqueous alkaline cleaning solution. These cleaning solutions are usually prepared by dissolving one or more strong alkalies in water, and are generally employed at elevated temperatures. The minor amount of aluminum or zinc powder in the trace amount of buffing composition which remains on the surface of the buffed or polished metal workpiece reacts violently with the hot aqueous alkaline cleaning solution to liberate gaseous hydrogen, which, in turn, causes the adhering buffing and polishing composition to separate from the metal surface. Particularly good results are obtained if the buffed workpiece containing the residual buffing composition is electrolytically cleaned in the aqueous alkaline cleaning solution by making the metal workpiece one of the electrodes in a direct current circuit. Under these conditions, the evolution of gaseous hydrogen on the metal surface is even more effective. This gaseous hydrogen functions as a scourer of the remaining traces of buffing composition adhering to the workpiece.

The following examples are illustrative of the various non-aqueous and aqueous buffing and polishing compositions which may be prepared in accordance with the invention:

25

## Example I

A non-aqueous buffing composition was prepared by uniformly blending 12.24 percent by weight of stearic acid, 10.70 percent by weight of saturated fatty acids (Hydrofol Glyceride No. 42), 1.05 percent by weight of wood rosin, 3.43 percent by weight of tallow oil, 1.09 percent by weight of No. 9 oil, 70.49 percent by weight of No. 6 lime, and 1 percent by weight of aluminum powder. This buffing composition is especially suitable for use as a nickel coloring compound, and may be easily and completely removed from the metal workpiece with an aqueous alkaline cleaning solution.

## Example II

A non-aqueous buffing composition was prepared by uniformly blending 18.85 percent by weight of saturated fatty acids (Hydrofol Acids B.G.), 3.19 percent by weight of tallow, 9.57 by weight of petrolatum, 18.05 percent by weight of No. 54 silica, 49.34 percent by weight of Rose Tripoli (once ground) and 1 percent by weight of aluminum powder. This composition is especially suitable for use in the cutting of non-ferrous metals, and may be easily and completely removed from the metal workpiece with an aqueous alkaline cleaning solution.

50

## Example III

A non-aqueous buffing composition suitable for use as a steel coloring compound was prepared by uniformly blending 18.75 percent by weight of stearic acid, 3.75 percent by weight of oleo stearine, 2.5 percent by weight of paraffin wax, 74 percent by weight of unfused alumina, and 1 percent by weight of aluminum powder. This composition is also easily and completely removed from a metal workpiece buffed with the composition merely by using an aqueous alkaline cleaning solution.

60

## Example IV

An aqueous buffing composition was prepared by emulsifying 5.5 parts by weight of saturated fatty acids, 1.5 parts by weight of triethanolamine, 0.9 part by weight of a surfactant (Triton X-100), 0.1 part by weight of a preservative, 3 parts by weight of petrolatum, 3 parts by weight of tallow, and 5 parts by weight of paraffin oil in 38.5 parts by weight of water. To this emulsion was then added 32 parts by weight of Rose Tripoli (once ground), 9.5 parts by weight of amorphous silica, and 1 part by weight of aluminum powder. The resultant aqueous

buffing composition is especially suitable for use as a cutting compound, and may be easily and completely removed from the metal workpiece with an aqueous alkaline cleaning solution.

*Example V*

An aqueous buffing composition suitable for use as a coloring compound was prepared by emulsifying 7 parts by weight of saturated fatty acids, 2 parts by weight of triethanolamine, 0.4 part by weight of a surfactant (Triton X-100), 0.1 part by weight of a preservative, 1 part by weight of paraffin oil, 1 part by weight oleo stearin, 10 parts by weight of amorphous silica, 31 parts by weight of aluminum oxide, and 1 part by weight of aluminum powder in 46.5 parts by weight of water. The resultant buffing composition is easily and completely removed from a metal workpiece buffed with the compound merely by using a minor amount (from about  $\frac{1}{2}$  to about 2

Although each of the foregoing examples of the invention show the use of aluminum powder in the buffing composition, equally satisfactory results may be obtained by using a minor amount (from about  $\frac{1}{2}$  to about 2 percent by weight) of zinc powder in the buffing composition. Consequently, the invention is applicable to any buffing composition comprising a carrier lubricant in which there is dispersed a major amount of an inorganic abrasive and a minor amount of either aluminum powder or zinc powder.

I claim:

1. A buffing composition consisting essentially of a carrier lubricant selected from the group consisting of grease, oil and soap, or mixtures thereof in an amount from about 10% to 32% by weight of the composition in which there is dispersed a major amount of an inorganic abrasive, characterized in that a metallic powder selected from the group consisting of aluminum and zinc in an amount from  $\frac{1}{2}\%$  to 2% by weight of the composition is dispersed in said lubricant.

2. A buffing composition consisting essentially of a carrier lubricant selected from the group consisting of grease, oil and soap, or mixtures thereof in an amount from about 10% to 32% by weight of the composition in which there is dispersed a major amount of an inorganic abrasive, characterized in that aluminum powder in an amount from  $\frac{1}{2}\%$  to 2% by weight of the composition is dispersed in said lubricant.

3. A buffing composition consisting essentially of a carrier lubricant selected from the group consisting of grease, oil and soap, or mixtures thereof in an amount from about 10% to 32% by weight of the composition in which there is dispersed a major amount of an inorganic abrasive, characterized in that zinc powder in an amount from  $\frac{1}{2}\%$  to 2% by weight of the composition is dispersed in said lubricant.

4. A non-aqueous buffing composition suitable for use as a nickel coloring compound comprising about 12 per-

cent by weight of stearic acid, about 11 percent by weight of a fatty glyceride, about 1 percent by weight of wood rosin, about 3½ percent by weight of tallow oil, about 70 percent by weight of finely divided lime, and about 1 percent by weight of aluminum powder.

5. A non-aqueous buffing composition suitable for use in cutting non-ferrous metals comprising about 19 percent by weight of saturated fatty acids, about 3 percent by weight of tallow, about 9½ percent by weight of petro-  
10 latum, about 18 percent by weight of finely divided silica, about 49 percent by weight of tripoli powder, and about 1 percent by weight of aluminum powder.

6. A non-aqueous buffing composition suitable for use as a steel coloring compound consisting essentially of about 19 percent by weight of stearic acid, about 4 percent by weight of oleo stearine, about 2½ percent by weight of a paraffinic wax, about 74 percent by weight of unfused alumina, and about 1 percent by weight of aluminum powder.

20 7. The buffing composition of claim 1 wherein said composition is arranged in an aqueous emulsion.

8. An aqueous buffing composition comprising about 5.5 parts by weight of a fatty acid, about 1.5 parts by weight of triethanolamine, about 0.9 part by weight of a surfactant, about 0.1 part by weight of a preservative, about 3 parts by weight of petro-  
25 latum, about 3 parts by weight of tallow, about 5 parts by weight of paraffin oil in 38.5 parts by weight of water, about 32 parts by weight of Rose Tripoli, about 9.5 parts by weight of amorphous silica and about 1 part by weight of aluminum powder.

9. An aqueous buffing composition suitable for use as a coloring compound comprising about 7 parts by weight of a saturated fatty acid, about 2 parts by weight of triethanolamine and about 0.4 part by weight of a surfactant, about 0.1 part by weight of a preservative, about 1 part by weight of paraffin oil, about 1 part by weight oleo stearine, about 10 parts by weight of amorphous silica, about 31 parts by weight of aluminum oxide and 1 part by weight of aluminum powder in 46.5 parts by weight of water.

**References Cited by the Examiner**

**UNITED STATES PATENTS**

|              |         |                |       |        |
|--------------|---------|----------------|-------|--------|
| 45 1,216,643 | 2/1917  | Yasuda         | ----- | 51—309 |
| 2,529,722    | 11/1950 | Chester        | ----- | 51—305 |
| 2,829,035    | 4/1958  | Doughty et al. | ----- | 51—304 |
| 2,889,215    | 6/1959  | Nelson         | ----- | 51—304 |

**FOREIGN PATENTS**

50 611,817 10/1926. France.

ALEXANDER H. BRODMERKEL, Primary Examiner.

55 D. J. ARNOLD, Assistant Examiner.